

## UNITED STATES PATENT OFFICE

ALBERT MELLOR AND DAVID TELFER MCLELLAN, OF SPONDON, NEAR DERBY, ENGLAND,  
ASSIGNORS TO CELANESE CORPORATION OF AMERICA, A CORPORATION OF DELA-  
WARE

## COLORATION OF TEXTILE MATERIAL

No Drawing. Application filed January 29, 1931, Serial No. 512,212, and in Great Britain April 2, 1930.

This invention relates to the production of uniform black colorations on mixed materials containing derivatives of cellulose and vegetable or other textile fibres.

5 A very widely used method for the production of black colorations on textile fibres is the oxidation of aniline on the material. By this means there may be very cheaply produced excellent blacks of exceptional fastness.

10 Considerable difficulties have, however, been encountered in the production of uniform aniline black shades on mixed materials containing cellulose derivatives and vegetable, animal or other textile fibres, since, 15 in general, the conditions necessary for the production of the best blacks on the cellulose derivative on the one hand and on the cellulosic or animal fibres on the other hand are not identical. Thus for example in addition 20 to the different affinities of cellulose acetate and cotton for aniline, the conditions for the oxidation of aniline to a good black on cotton are very different from the conditions 25 required for the production of a good black on cellulose acetate.

According to the present invention uniform black colorations are obtained on mixed materials containing derivatives of cellulose 30 and other textile fibres by first causing the mixed material to absorb para-aminodiphenylamine or a derivative thereof, and then mechanically impregnating it with aniline or its homologues or compounds thereof and 35 oxidizing.

By such a process the para-aminodiphenylamine or the like is preferentially absorbed substantively by the cellulose derivative, while both or all the constituents of the 40 mixed materials are impregnated with aniline or the like.

The diphenylamine base may be absorbed substantively from solution or dispersion. Advantageously solutions may, prior to application, be made acid by means of suitable acids, preferably organic acids, e. g. lactic acid or acetic acid. The substantive treatment is preferably given however, with the diphenylamine base in dispersion. Thus for 45 example the mixed fabric may be immersed

in a bath containing p-aminodiphenylamine or 2:4-diaminodiphenylamine dispersed by means of Turkey red oil.

After the substantive treatment the materials may be scoured, washed and dried, 55 padded, sprayed, or otherwise mechanically impregnated with aniline, aniline hydrochloride or other compound of aniline or the like, and then treated with an oxidizing agent or mixture, or the oxidizing agent or mixture 60 may be applied together with the aniline etc. After impregnation, the materials may be dried, aged, and if desired, chromed, or subjected to any other desired after-treatment.

If desired, instead of applying to the material the diphenylamine base the latter may 65 be produced on the material. Thus for example 2:4-dinitrodiphenylamine or other p-nitrodiphenylamine may be applied to the mixed material and then reduced on the material to give the amino body. 70

The absorption of the diphenylamine base or other diphenylamine body and the compound of aniline or homologues of aniline into the cellulose derivative fibre may be 75 promoted by means of alcohol, hydroquinone, or other substance having a swelling action on the fibre. The oxidizing agent or mixture employed for the production of a black may contain a chlorate, hypochlorite, bi- 80 chromate, or other suitable oxidizing agent, and may also contain one or more catalysts or oxygen carriers, e. g. salts of vanadium, copper, iron or chromium. The development of the color may also be assisted by 85 means of aluminium chloride or any other suitable inorganic assistant.

The following example illustrates carrying the invention into effect, but it is to be understood that it is in no way limitative:— 90

100 pounds of a mixed fabric containing cotton and cellulose acetate are scoured at 60° C. on a dye jig in a 30 to 1 bath containing 1 gram per litre of soap and 2 ccs. per litre Turkey red oil. After half an hour 95 10 pounds of a 10 per cent. dispersion of para-aminodiphenylamine in Turkey red oil is added to the scouring bath, and the fabric treated for a further half an hour at 80° to 85° C.; at the close of this period the fabric 100

is washed in warm water, hydroextracted and dried. It is then padded in an aniline liquor made up as follows:—

- 84 pounds aniline hydrochloride, 18 pounds 5 potassium chloride, 18 pounds crystallized copper sulphate, water to make 80 gallons. The material is finally dried, aged at 45° to 50° C. and chromed with 1 to 3° Tw. sodium bichromate at ordinary temperatures for one 10 hour. An excellent uniform black is thus obtained on the material.

The process of the present invention aims more particularly at producing uniform blacks on mixed materials comprising a cellulose derivative and cotton, linen, regenerated cellulose, artificial silks or rayons, or other cellulosic fibres. It is however of considerable use in the production of uniform blacks on mixed materials comprising cellulose 15 derivatives and animal fibres, for example, natural silk. The mixed material may contain any organic derivative of cellulose. Thus for example the material may contain cellulose acetate as already mentioned, or it 20 may contain other organic esters of cellulose, e. g. cellulose formate, propionate, butyrate, or the products obtainable by the treatment of alkalinized cellulose with an esterifying agent, e. g. the product known as "immunized cotton" obtained by treating alkalinized cellulose with para-toluene sulphochloride. Again, the material may contain cellulose 25 ethers, for example methyl, ethyl or benzyl cellulose or the corresponding condensation 30 products of cellulose and glycols, or other polyhydric alcohols.

What we claim and desire to secure by Letters Patent is:—

1. Process for the production of black colorations on mixed materials containing derivatives of cellulose and cellulosic fibres, comprising causing the cellulose derivatives to absorb a compound selected from the group consisting of para-aminodiphenylamine and 40 its derivatives, mechanically impregnating the mixed material with a substance selected from the group consisting of aniline, its homologues, and its compounds, and subjecting the material to the action of an oxidizing agent.

2. Process for the production of black colorations on mixed materials containing cellulose acetate and cellulosic fibres, comprising causing the cellulose acetate to absorb a compound selected from the group consisting of para-aminodiphenylamine and its derivatives, mechanically impregnating the mixed material with a substance selected from the group consisting of aniline, its homologues, 55 and its compounds, and subjecting the material to the action of an oxidizing agent.

3. Process for the production of black colorations on mixed materials containing cellulose acetate and cotton, comprising causing the cellulose acetate to absorb a compound

selected from the group consisting of para-aminodiphenylamine and its derivatives, mechanically impregnating the mixed material with a substance selected from the group consisting of aniline, its homologues and its compounds, and subjecting the material to the action of an oxidizing agent.

4. Process for the production of black colorations on mixed materials containing derivatives of cellulose and cellulosic fibres, comprising causing the cellulose derivative to absorb a compound of the group consisting of para-aminodiphenylamine and its derivatives from an aqueous dispersion of said compound, mechanically impregnating the mixed material with a compound selected from the group consisting of aniline, its homologues, and its compounds, and subjecting the materials to the action of an oxidizing agent.

5. Process for the production of black colorations on mixed materials containing cellulose acetate and cellulosic fibres comprising causing the cellulose acetate to absorb a compound of the group consisting of para-aminodiphenylamine and its derivatives from an aqueous dispersion of said compound, mechanically impregnating the mixed material with a compound selected from the group consisting of aniline, its homologues and its compounds, and subjecting the material to the action of an oxidizing agent.

6. Process for the production of black colorations on mixed materials containing derivatives of cellulose and cellulosic fibres, comprising producing on the cellulose derivative fibre a para-aminodiphenylamine by reduction of the corresponding nitro compound, mechanically impregnating the mixed material with a compound selected from the group consisting of aniline, its homologues and its compounds, and subjecting the material to the action of an oxidizing agent.

In testimony whereof we have hereunto subscribed our names.

ALBERT MELLOR.

DAVID TELFER McLELLAN.

110

100

105

115

120

125

130

70

75

80

85

90

95

100

105

110